



US006497997B2

(12) **United States Patent**  
Simons

(10) **Patent No.:** US 6,497,997 B2  
(45) **Date of Patent:** Dec. 24, 2002

(54) **METHOD AND MATERIAL FOR  
PHOTOGRAPHIC PROCESSING**

6,022,673 A \* 2/2000 Ishikawa ..... 430/351  
6,083,668 A \* 7/2000 Matsumoto et al. ..... 430/206

(75) Inventor: **Michael J. Simons**, Eastcote (GB)

FOREIGN PATENT DOCUMENTS

(73) Assignee: **Eastman Kodak Company**, Rochester,  
NY (US)

WO 93/12462 6/1993

(\*) Notice: Subject to any disclaimer, the term of this  
patent is extended or adjusted under 35  
U.S.C. 154(b) by 0 days.

\* cited by examiner

(21) Appl. No.: **09/874,884**

(22) Filed: **Jun. 5, 2001**

(65) **Prior Publication Data**

US 2002/0009678 A1 Jan. 24, 2002

(30) **Foreign Application Priority Data**

Jun. 13, 2000 (GB) ..... 0014422

(51) **Int. Cl.<sup>7</sup>** ..... G03C 5/38; G03C 7/42

(52) **U.S. Cl.** ..... 430/429; 430/372; 430/404

(58) **Field of Search** ..... 430/404, 428,  
430/429, 372

(56) **References Cited**

U.S. PATENT DOCUMENTS

4,775,614 A \* 10/1988 De Rycke ..... 430/203

*Primary Examiner*—Hoa Van Le

(74) *Attorney, Agent, or Firm*—Chris P. Konkol

(57) **ABSTRACT**

A method of providing an image in an imagewise exposed photographic silver halide material comprising at least one silver halide emulsion layer, which method comprises developing the silver halide and fixing the remaining silver halide by contacting it with a molten composition comprising a silver halide complexing agent which is present in sufficient amount to render the silver halide substantially clear. The photographic silver halide material may comprise at least one silver halide emulsion layer on a support wherein the material also comprises a layer of a composition comprising a silver halide complexing agent which is liquefiable by heat and which, when molten, is in reactive association with the silver halide. The image formed may be scanned to produce an electronic rendition of the image.

**10 Claims, 2 Drawing Sheets**





FIG. 2

## METHOD AND MATERIAL FOR PHOTOGRAPHIC PROCESSING

### FIELD OF THE INVENTION

The invention relates to a method and material for photographic processing.

### BACKGROUND OF THE INVENTION

The basic image-forming process of photography comprises the exposure of a silver halide photographic recording material, such as a color film, to electromagnetic radiation, and the chemical processing of the exposed material to provide a useful image. Chemical processing involves two fundamental steps. The first is treatment of the exposed silver halide material with a developing agent wherein some or all of the silver ion is reduced to metallic silver, and in the case of color materials, a dye image is formed (because of a color developing agent).

For color materials, the second fundamental step is the removal of silver metal by one or more steps of bleaching and fixing so that only a dye image remains in the processed material. During bleaching, the developed silver is oxidized to a silver salt by a suitable bleaching agent. The oxidized silver is then dissolved and removed from the material using a "fixing" agent or silver solvent in a fixing step. Black-and-white materials are desilvered using only the fixing step.

Additional photoprocessing steps may be needed including rinsing or dye stabilization that require even more photoprocessing chemicals. In the case of color reversal materials, additional photoprocessing steps include black-and-white development, a reversal step, pre-bleaching or conditioning step and one or more rinsing steps.

All of these photoprocessing steps require preparation of the photoprocessing compositions (whether in aqueous or solid form), large or small photoprocessing tanks or reservoirs to hold the compositions, and disposal or regeneration of the "spent" compositions once a predetermined amount of exposed material has been processed. All of these operations require considerable manufacturing effort, shipping and handling of chemicals and aqueous solutions, replenishment of the solutions, and disposal of solutions into the environment. These characteristics of conventional photoprocessing are labor intensive, tedious, costly and potentially harmful to the environment (although much work has been accomplished in the industry to make the compositions more environmentally "friendly").

New business opportunities are thought to exist if ways can be found to minimize or obviate the problems described above. Providing photographic images (often known as "photofinishing") is a growing business and yet there is a need to provide those images in ways that do not require some or all of the traditional photoprocessing solutions, equipment and replenishment systems.

As noted above, a fixing step is commonly employed in photographic processing. WO 93/12462 describes a method of fixing a developed photographic silver halide material comprising at least two silver halide layers sensitised to different regions of the spectrum, comprising placing the material in face-to-face contact with a fixer sheet in the presence of a processing solution and a silver halide solvent which forms a solubilised silver halide species from the undeveloped areas of the material, wherein the fixer sheet contains reducing means capable of forming metallic silver therein from the solubilised silver halide.

Recent digital technologies in the photographic industry offer advantages in that they can enable the user to manipulate the images after photochemical processing by scanning to create a digital representation of the image. One of these advantages is the ability to readjust the exposure by automatic tone scaling to correct for either over- or underexposure. Other uses of digitization are to crop, enlarge or otherwise modify the image, or to send the image to other users electronically for various purposes. The growing awareness of digitization of photographic images provides almost limitless possibilities for image manipulation for various purposes in a number of industries.

### PROBLEM TO BE SOLVED BY THE INVENTION

A method of fixing or clearing a photographic material is required that may be done in a substantially dry condition, that is without water having to be provided in addition to the fixing agent. Unlike conventional fixing, there is no requirement for the silver complex formed to be removed from the emulsion layer.

### SUMMARY OF THE INVENTION

The invention relates to a method of providing an image in an imagewise exposed photographic silver halide material comprising at least one silver halide emulsion layer, the method comprising developing the silver halide and fixing the remaining silver halide by contacting it with a molten composition comprising a silver halide complexing agent which is present in sufficient amount to render the silver halide substantially clear.

In another aspect, the invention relates to a photographic silver halide material comprising at least one silver halide emulsion layer on a support wherein the material also comprises a layer of a composition comprising a silver halide complexing agent which is liquefiable by heat and which, when molten, is in reactive association with the silver halide.

### ADVANTAGEOUS EFFECT OF THE INVENTION

The invention provides a rapid means of processing photographic films which may subsequently be scanned. The silver halide grains are rendered non-scattering or transparent to light by dissolving the light scattering silver halide. The image is rendered more stable to subsequent light exposure. Scanner light may pass readily through the film and the level of optical noise reduced. The present invention allows the film to be rendered transparent by means of a simple, dry lamination and heating step.

### BRIEF DESCRIPTION OF THE DRAWINGS

FIG. 1 shows in block diagram form an apparatus for processing and viewing image information obtained by scanning the color negative materials.

FIG. 2 is a block diagram showing electronic signal processing of the input trichromatic image-bearing signals derived from scanning a color negative recording material.

### DETAILED DESCRIPTION OF THE INVENTION

The method of the invention comprises developing the imagewise exposed silver halide material and fixing the remaining i.e. non-developed silver halide by contacting it with a molten composition comprising a silver halide com-

plexing agent which is present in sufficient amount to render the silver halide substantially clear.

Preferably, the silver halide and the composition comprising the silver halide complexing agent are brought into contact at a temperature from 40 to 170° C., more preferably at a temperature from 70 to 150° C. Preferably, the composition comprising the silver halide complexing agent has melting point within the given temperature ranges.

The silver complexing agent may be a heterocyclic amine.

Preferably, the heterocyclic amine is a substituted or unsubstituted imidazole, pyrazole or triazole.

Particularly preferred silver complexing agents include imidazole and alkyl substituted imidazoles e.g. 2-methyl imidazole, 4-methyl imidazole, and 1,2-dimethyl imidazole.

Examples of other suitable heterocyclic amine silver complexing agents include benzimidazole; 1,2,4-triazole and substituted 1,2,4-triazoles e.g. 4-amino-1,2,4-triazole, 3-amino-1,2,4-triazole and 1,2,4-triazole-3-thiol; pyrazole; and 1-(hydroxyethyl)-tetrahydrotriazine-4-thiol.

Examples of other silver complexing agents include sodium thiocyanate dihydrate and ammonium thiocyanate and thiourea.

The silver complexing agents may be used with a compound which co-melts with the complexing agent to provide a molten mixture in the desired temperature range. Examples of compounds which may be suitable as co-melters for the organic complexing agents listed above include amides such as benzamide (m.pt. 129° C.), p-toluanide (m.pt. 162° C.), anthranilamide (m.pt. 113° C.), salicylamide (m.pt. 142° C.), nicotinamide (m.pt. 131° C.), ureas such as 1,3-dimethylurea (m.pt. 102° C.) and n-butylurea (m.pt. 94° C.), and other compounds such as antipyrine (m.pt. 112° C.), coumarin (m.pt. 71° C.), cyclohexane-1,4-diol (m.pt. 99° C.), p-acetophenetidite (m.pt. 136° C.), succinimide (m.pt. 125° C.), and polyethylene glycols (various melting points, depending on molecular weight).

The silver complexing agent may be present in an amount from 2 to 200 g/m<sup>2</sup>, preferably from 5 to 75 g/m<sup>2</sup>.

It is advantageous for the silver halide complexing agent to render the silver halide substantially clear in a short a time period as possible. The complexing agents described above have a clearing effect in 60s or less. Preferred complexing agents have a clearing effect in 20s or less, most preferably 5s or less.

The composition comprising a silver halide complexing agent may be initially located in a separate fixer sheet which is brought into contact with the photographic silver halide material and heated to render the composition molten. For example, the fixer sheet may be laminated to the exposed and developed photographic silver halide material. Heating of the laminate melts the composition comprising a silver halide complexing agent which is in reactive association with the silver halide i.e. the silver halide complexing agent can diffuse into the emulsion layer and react with the silver halide. If desired, the fixer sheet may be releasably laminated to the photographic material so that, after use, the sheet may be delaminated.

Alternatively, the composition of the silver halide complexing agent may be initially located in an integral layer of the photographic silver halide material on the same side of the support as the silver halide photographic layer.

Preferably, the fixer sheet comprises a layer of the composition comprising the silver halide complexing agent in a polymeric binder on a support. Suitable polymeric binders

include high molecular weight materials and resins such as poly(vinyl butyral), cellulose acetate butyrate, poly(methylmethacrylate), poly(vinylpyrrolidone), ethyl cellulose, polystyrene, poly(vinylchloride), chlorinated rubbers, polychloroprene, polyisoprene, polyisobutylene, butadiene-styrene copolymers, polyvinyl acetate, copolymers of vinyl chloride and vinyl acetate, copolymers of vinylidene chloride and vinyl acetate, polyvinylpyridines, and polycarbonates. Water-soluble resins and polymers include gelatin, poly(vinyl alcohol), polyacrylamide, polyethylene glycols, polyethylene oxide, hydroxyethylcellulose, hydroxypropylcellulose, carboxymethylcellulose, polyacrylic acid, polyacrylamide, copolymers of acrylic acid with ethylene or styrene, poly(styrenesulfonic acid-co-maleic acid) salts, and naturally occurring materials such as agar, gum acacia, gum arabic, and caragenin.

Suitable supports include those commonly used for photographic materials e.g. polyethylene terephthalate and numerous examples are disclosed in Section XV of *Research Disclosure*, September 1996, Number 389, Item 38957, September 1996, Number 389, Item 38957 (hereafter referred to as ("Research Disclosure I"). All sections referred to herein are sections of *Research Disclosure I*, unless otherwise indicated. (All Research Disclosures referenced herein are published by Kenneth Mason Publications, Ltd., Dudley Annex, 12a North Street, Emsworth, Hampshire PO10 7DQ, ENGLAND). Preferably, the support is transparent.

Fixer sheets may be prepared by coating the support with a coating composition comprising the silver halide complexing agent.

The coating composition may be coated from a suitable solvent which will dissolve both the silver complexing agent and the binder. Depending on the substances to be coated, the solvent could be for example water, or an organic solvent such as acetone, methyl ethyl ketone, butanone, ethyl acetate, methanol, ethanol, chlorinated hydrocarbons, or suitable mixtures thereof.

Any conventional coating method may be employed e.g. coating procedures known in the photographic art, including dip coating, air knife coating, curtain coating or extrusion coating using hoppers. If desired, two or more layers are coated simultaneously.

In a preferred embodiment, a polymeric binder is dissolved in the molten silver complexing agent e.g. imidazole at a temperature above its melting point and the molten composition is extruded onto a suitable support.

The imidazole silver complexing agents noted above are mildly basic and it may be desirable to use them in combination with acid substances to reduce the basicity. Suitable acid substances include succinic acid, citric acid, benzoic acid and salicylic acid.

It may also be desirable to use development restrainers in combination with the silver complexing agent to prevent physical development of the silver complex formed. Suitable development restrainers include simple bromides e.g. ammonium bromide and lithium bromide, which are soluble in non-aqueous solvents, and also organic restrainers e.g. benzotriazoles, 3-mercaptoptriazoles and phenyl mercaptotetrazoles.

The method and material of the invention may be used in any form of photographic system e.g. color or black and white. In a preferred embodiment of the invention the photographic material used is a color negative film. Prints can be made from the film by conventional optical tech-

niques or by scanning the film and printing using a laser, light emitting diode or a cathode ray tube.

A color negative film construction useful in the practice of the invention is illustrated by the following element, SCN-1:

| Element SCN-I |                            |
|---------------|----------------------------|
| SOC           | Surface Overcoat           |
| BU            | Blue Recording Layer Unit  |
| IL1           | First Interlayer           |
| GU            | Green Recording Layer Unit |
| IL2           | Second Interlayer          |
| RU            | Red Recording Layer Unit   |
| AHU           | Antihalation Layer Unit    |
| S             | Support                    |
| SOC           | Surface Overcoat           |

The support S can be either reflective or transparent, which is usually preferred. When reflective, the support is white and can take the form of any conventional support currently employed in color print elements. When the support is transparent, it can be colorless or tinted and can take the form of any conventional support currently employed in color negative elements—e.g., a colorless or tinted transparent film support. Details of support construction are well understood in the art. Examples of useful supports are poly(vinyl acetal) film, polystyrene film, poly(ethyleneterephthalate) film, poly(ethylene naphthalate) film, polycarbonate film, and related films and resinous materials, as well as paper, cloth, glass, metal, and other supports that withstand the anticipated processing conditions. The element can contain additional layers, such as filter layers, interlayers, overcoat layers, subbing layers, antihalation layers and the like. Transparent and reflective support constructions, including subbing layers to enhance adhesion, are disclosed in Section XV of *Research Disclosure I*.

Photothermographic elements of the present invention may also usefully include a magnetic recording material as described in *Research Disclosure*, Item 34390, November 1992, or a transparent magnetic recording layer such as a layer containing magnetic particles on the underside of a transparent support as in U.S. Pat. No. 4,279,945, and U.S. Pat. No. 4,302,523.

Each of blue, green and red recording layer units BU, GU and RU are formed of one or more hydrophilic colloid layers and contain at least one radiation-sensitive silver halide emulsion and coupler, including at least one dye image-forming coupler. It is preferred that the green, and red recording units are subdivided into at least two recording layer sub-units to provide increased recording latitude and reduced image granularity. In the simplest contemplated construction each of the layer units or layer sub-units consists of a single hydrophilic colloid layer containing emulsion and coupler. When coupler present in a layer unit or layer sub-unit is coated in a hydrophilic colloid layer other than an emulsion containing layer, the coupler containing hydrophilic colloid layer is positioned to receive oxidized color developing agent from the emulsion during development. Usually the coupler containing layer is the next adjacent hydrophilic colloid layer to the emulsion containing layer.

In order to ensure excellent image sharpness, and to facilitate manufacture and use in cameras, all of the sensitized layers are preferably positioned on a common face of

the support. When in spool form, the element will be spooled such that when unspooled in a camera, exposing light strikes all of the sensitized layers before striking the face of the support carrying these layers. Further, to ensure excellent sharpness of images exposed onto the element, the total thickness of the layer units above the support should be controlled. Generally, the total thickness of the sensitized layers, interlayers and protective layers on the exposure face of the support are less than 35  $\mu\text{m}$ .

Any convenient selection from among conventional radiation-sensitive silver halide emulsions can be incorporated within the layer units. Most commonly high bromide emulsions containing a minor amount of iodide are employed. To realize higher rates of processing, high chloride emulsions can be employed. Radiation-sensitive silver chloride, silver bromide, silver iodobromide, silver iodochloride, silver chlorobromide, silver bromochloride, silver iodochlorobromide and silver iodobromochloride grains are all contemplated. The grains can be either regular or irregular (e.g., tabular). Tabular grain emulsions, those in which tabular grains account for at least 50 (preferably at least 70 and optimally at least 90) percent of total grain projected area are particularly advantageous for increasing speed in relation to granularity. To be considered tabular a grain requires two major parallel faces with a ratio of its equivalent circular diameter (ECD) to its thickness of at least 2. Specifically preferred tabular grain emulsions are those having a tabular grain average aspect ratio of at least 5 and, optimally, greater than 8. Preferred mean tabular grain thicknesses are less than 0.3  $\mu\text{m}$  (most preferably less than 0.2  $\mu\text{m}$ ). Ultrathin tabular grain emulsions, those with mean tabular grain thicknesses of less than 0.07  $\mu\text{m}$ , are specifically contemplated. The grains preferably form surface latent images so that they produce negative images when processed in a surface developer in color negative film forms of the invention.

Illustrations of conventional radiation-sensitive silver halide emulsions are provided by *Research Disclosure I*, cited above, I. Emulsion grains and their preparation.

Chemical sensitization of the emulsions, which can take any conventional form, is illustrated in section IV. Chemical sensitization. Compounds useful as chemical sensitizers, include, for example, active gelatin, sulfur, selenium, tellurium, gold, platinum, palladium, iridium, osmium, rhenium, phosphorous, or combinations thereof. Chemical sensitization is generally carried out at pAg levels of from 5 to 10, pH levels of from 4 to 8, and temperatures of from 30 to 80° C. Spectral sensitization and sensitizing dyes, which can take any conventional form, are illustrated by section V. Spectral sensitization and desensitization. The dye may be added to an emulsion of the silver halide grains and a hydrophilic colloid at any time prior to (e.g., during or after chemical sensitization) or simultaneous with the coating of the emulsion on a photographic element. The dyes may, for example, be added as a solution in water or an alcohol or as a dispersion of solid particles. The emulsion layers also typically include one or more antifoggants or stabilizers, which can take any conventional form, as illustrated by section VII. Antifoggants and stabilizers.

The silver halide grains to be used in the invention may be prepared according to methods known in the art, such as those described in *Research Disclosure I*, cited above, and James, *The Theory of the Photographic Process*. These include methods such as ammoniacal emulsion making, neutral or acidic emulsion making, and others known in the art. These methods generally involve mixing a water soluble silver salt with a water soluble halide salt in the presence of

a protective colloid, and controlling the temperature, pAg, pH values, etc, at suitable values during formation of the silver halide by precipitation.

In the course of grain precipitation one or more dopants (grain occlusions other than silver and halide) can be introduced to modify grain properties. For example, any of the various conventional dopants disclosed in *Research Disclosure I*, Section I. Emulsion grains and their preparation, sub-section G. Grain modifying conditions and adjustments, paragraphs (3), (4) and (5), can be present in the emulsions of the invention. In addition it is specifically contemplated to dope the grains with transition metal hexacoordination complexes containing one or more organic ligands, as taught by Olm et al U.S. Pat. No. 5,360,712.

It is specifically contemplated to incorporate in the face centered cubic crystal lattice of the grains a dopant capable of increasing imaging speed by forming a shallow electron trap (hereinafter also referred to as a SET) as discussed in *Research Disclosure* Item 36736 published November 1994.

The photographic elements of the present invention, as is typical, provide the silver halide in the form of an emulsion. Photographic emulsions generally include a vehicle for coating the emulsion as a layer of a photographic element. Useful vehicles include both naturally occurring substances such as proteins, protein derivatives, cellulose derivatives (e.g., cellulose esters), gelatin (e.g., alkali-treated gelatin such as cattle bone or hide gelatin, or acid treated gelatin such as pigskin gelatin), deionized gelatin, gelatin derivatives (e.g., acetylated gelatin, phthalated gelatin, and the like), and others as described in *Research Disclosure*, I. Also useful as vehicles or vehicle extenders are hydrophilic water-permeable colloids. These include synthetic polymeric peptizers, carriers, and/or binders such as poly(vinyl alcohol), poly(vinyl lactams), acrylamide polymers, polyvinyl acetals, polymers of alkyl and sulfoalkyl acrylates and methacrylates, hydrolyzed polyvinyl acetates, polyamides, polyvinyl pyridine, methacrylamide copolymers. The vehicle can be present in the emulsion in any amount useful in photographic emulsions. The emulsion can also include any of the addenda known to be useful in photographic emulsions.

While any useful quantity of light sensitive silver, as silver halide, can be employed in the elements useful in this invention, it is preferred that the total quantity be less than 10 g/m<sup>2</sup> of silver. Silver quantities of less than 7 g/m<sup>2</sup> are preferred, and silver quantities of less than 5 g/m<sup>2</sup> are even more preferred. The lower quantities of silver improve the optics of the elements, thus enabling the production of sharper pictures using the elements. These lower quantities of silver are additionally important in that they enable rapid development and clearing of the elements. Conversely, a silver coating coverage of at least 1.5 g of coated silver per m<sup>2</sup> of support surface area in the element is necessary to realize an exposure latitude of at least 2.7 log E while maintaining an adequately low graininess position for pictures intended to be enlarged.

BU contains at least one yellow dye image-forming coupler, GU contains at least one magenta dye image-forming coupler, and RU contains at least one cyan dye image-forming coupler. Any convenient combination of conventional dye image-forming couplers can be employed. Conventional dye image-forming couplers are illustrated by *Research Disclosure* I, cited above, X. Dye image formers and modifiers, B. Image-dye-forming couplers. The photographic elements may further contain other image-modifying compounds such as "Development Inhibitor-

Releasing" compounds (DIR's). Useful additional DIR's for elements of the present invention, are known in the art and examples are described in U.S. Pat. Nos. 3,137,578; 3,148,022; 3,148,062; 3,227,554; 3,384,657; 3,379,529; 3,615,506; 3,617,291; 3,620,746; 3,701,783; 3,733,201; 4,049,455; 4,095,984; 4,126,459; 4,149,886; 4,150,228; 4,211,562; 4,248,962; 4,259,437; 4,362,878; 4,409,323; 4,477,563; 4,782,012; 4,962,018; 4,500,634; 4,579,816; 4,607,004; 4,618,571; 4,678,739; 4,746,600; 4,746,601; 4,791,049; 4,857,447; 4,865,959; 4,880,342; 4,886,736; 4,937,179; 4,946,767; 4,948,716; 4,952,485; 4,956,269; 4,959,299; 4,966,835; 4,985,336 as well as in patent publications GB 1,560,240; GB 2,007,662; GB 2,032,914; GB 2,099,167; DE 2,842,063, DE 2,937,127; DE 3,636,824; DE 3,644,416 as well as the following European Patent Publications: 272,573; 335,319; 336,411; 346,899; 362,870; 365,252; 365,346; 373,382; 376,212; 377,463; 378,236; 384,670; 396,486; 401,612; 401,613.

DIR compounds are also disclosed in "Developer-Inhibitor-Releasing (DIR) Couplers for Color Photography," C. R. Barr, J. R. Thirtle and P. W. Vittum in *Photographic Science and Engineering*, Vol. 13, p. 174 (1969).

It is common practice to coat one, two or three separate emulsion layers within a single dye image-forming layer unit. When two or more emulsion layers are coated in a single layer unit, they are typically chosen to differ in sensitivity. When a more sensitive emulsion is coated over a less sensitive emulsion, a higher speed is realized than when the two emulsions are blended. When a less sensitive emulsion is coated over a more sensitive emulsion, a higher contrast is realized than when the two emulsions are blended. It is preferred that the most sensitive emulsion be located nearest the source of exposing radiation and the slowest emulsion be located nearest the support.

One or more of the layer units of the invention is preferably subdivided into at least two, and more preferably three or more sub-unit layers. It is preferred that all light sensitive silver halide emulsions in the color recording unit have spectral sensitivity in the same region of the visible spectrum. In this embodiment, while all silver halide emulsions incorporated in the unit have spectral absorptance according to invention, it is expected that there are minor differences in spectral absorptance properties between them. In still more preferred embodiments, the sensitizations of the slower silver halide emulsions are specifically tailored to account for the light shielding effects of the faster silver halide emulsions of the layer unit that reside above them, in order to provide an imagewise uniform spectral response by the photographic recording material as exposure varies with low to high light levels. Thus higher proportions of peak light absorbing spectral sensitizing dyes may be desirable in the slower emulsions of the subdivided layer unit to account for on-peak shielding and broadening of the underlying layer spectral sensitivity.

The interlayers IL1 and IL2 are hydrophilic colloid layers having as their primary function color contamination reduction i.e. prevention of oxidized developing agent from migrating to an adjacent recording layer unit before reacting with dye-forming coupler. The interlayers are in part effective simply by increasing the diffusion path length that oxidized developing agent must travel. To increase the effectiveness of the interlayers to intercept oxidized developing agent, it is conventional practice to incorporate oxidized developing agent. Antistain agents (oxidized developing agent scavengers) can be selected from among those disclosed by *Research Disclosure* I, X. Dye image formers and modifiers, D. Hue modifiers/stabilization, paragraph (2).

When one or more silver halide emulsions in GU and RU are high bromide emulsions and, hence have significant native sensitivity to blue light, it is preferred to incorporate a yellow filter, such as Carey Lea silver or a yellow processing solution decolorizable dye, in IL1. Suitable yellow filter dyes can be selected from among those illustrated by *Research Disclosure*, Section VIII. Absorbing and scattering materials, B. Absorbing materials. In some elements, magenta colored filter materials are absent from IL2 and RU.

The antihalation layer unit AHU typically contains a processing solution removable or decolorizable light absorbing material, such as one or a combination of pigments and dyes. Suitable materials can be selected from among those disclosed in *Research Disclosure* I, Section VIII. Absorbing materials. A common alternative location for AHU is between the support S and the recording layer unit coated nearest the support.

The surface overcoats SOC are hydrophilic colloid layers that are provided for physical protection of the color negative elements during handling and processing. Each SOC also provides a convenient location for incorporation of addenda that are most effective at or near the surface of the color negative element. In some instances the surface overcoat is divided into a surface layer and an interlayer, the latter functioning as spacer between the addenda in the surface layer and the adjacent recording layer unit. In another common variant form, addenda are distributed between the surface layer and the interlayer, with the latter containing addenda that are compatible with the adjacent recording layer unit. Most typically the SOC contains addenda, such as coating aids, plasticizers and lubricants, antistats and matting agents, such as illustrated by *Research Disclosure* I, Section IX. Coating physical property modifying addenda. The SOC overlying the emulsion layers additionally preferably contains an ultraviolet absorber, such as illustrated by *Research Disclosure* I, Section VI. UV dyes/optical brighteners/luminescent dyes, paragraph (1).

Instead of the layer unit sequence of element SCN-1, alternative layer units sequences can be employed and are particularly attractive for some emulsion choices. Using high chloride emulsions and/or thin (<0.2  $\mu\text{m}$  mean grain thickness) tabular grain emulsions all possible interchanges of the positions of BU, GU and RU can be undertaken without risk of blue light contamination of the minus blue records, since these emulsions exhibit negligible native sensitivity in the visible spectrum. For the same reason, it is unnecessary to incorporate blue light absorbers in the interlayers.

When the emulsion layers within a dye image-forming layer unit differ in speed, it is conventional practice to limit the incorporation of dye image-forming coupler in the layer of highest speed to less than a stoichiometric amount, based on silver. The function of the highest speed emulsion layer is to create the portion of the characteristic curve just above the minimum density-i.e., in an exposure region that is below the threshold sensitivity of the remaining emulsion layer or layers in the layer unit. In this way, adding the increased granularity of the highest sensitivity speed emulsion layer to the dye image record produced is minimized without sacrificing imaging speed.

In the foregoing discussion the blue, green and red recording layer units are described as containing yellow, magenta and cyan image dye-forming couplers, respectively, as is conventional practice in color negative elements used for printing. The invention can be suitably applied to conventional color negative construction as illus-

trated. Color reversal film construction would take a similar form, with the exception that colored masking couplers would be completely absent; in typical forms, development inhibitor releasing couplers would also be absent. In preferred embodiments, the color negative elements are intended exclusively for scanning to produce three separate electronic color records. Thus the actual hue of the image dye produced is of no importance. What is essential is merely that the dye image produced in each of the layer units be differentiable from that produced by each of the remaining layer units. To provide this capability of differentiation it is contemplated that each of the layer units contain one or more dye image-forming couplers chosen to produce image dye having an absorption half-peak bandwidth lying in a different spectral region. It is immaterial whether the blue, green or red recording layer unit forms a yellow, magenta or cyan dye having an absorption half peak bandwidth in the blue, green or red region of the spectrum, as is conventional in a color negative element intended for use in printing, or an absorption half-peak bandwidth in any other convenient region of the spectrum, ranging from the near ultraviolet (300–400 nm) through the visible and through the near infrared (700–1200 nm), so long as the absorption half-peak bandwidths of the image dye in the layer units extend over substantially non-coextensive wavelength ranges. The term “substantially non-coextensive wavelength ranges” means that each image dye exhibits an absorption half-peak band width that extends over at least a 25 (preferably 50) nm spectral region that is not occupied by an absorption half-peak band width of another image dye. Ideally the image dyes exhibit absorption half-peak band widths that are mutually exclusive.

When a layer unit contains two or more emulsion layers differing in speed, it is possible to lower image granularity in the image to be viewed, recreated from an electronic record, by forming in each emulsion layer of the layer unit a dye image which exhibits an absorption half-peak band width that lies in a different spectral region than the dye images of the other emulsion layers of layer unit. This technique is particularly well suited to elements in which the layer units are divided into sub-units that differ in speed. This allows multiple electronic records to be created for each layer unit, corresponding to the differing dye images formed by the emulsion layers of the same spectral sensitivity. The digital record formed by scanning the dye image formed by an emulsion layer of the highest speed is used to recreate the portion of the dye image to be viewed lying just above minimum density. At higher exposure levels second and, optionally, third electronic records can be formed by scanning spectrally differentiated dye images formed by the remaining emulsion layer or layers. These digital records contain less noise (lower granularity) and can be used in recreating the image to be viewed over exposure ranges above the threshold exposure level of the slower emulsion layers. This technique for lowering granularity is disclosed in greater detail by Sutton U.S. Pat. No. 5,314,794.

Each layer unit of the color negative elements of the invention produces a dye image characteristic curve gamma of less than 1.5, which facilitates obtaining an exposure latitude of at least 2.7 log E. A minimum acceptable exposure latitude of a multicolor photographic element is that which allows accurately recording the most extreme whites (e.g., a bride's wedding gown) and the most extreme blacks (e.g., a bride groom's tuxedo) that are likely to arise in photographic use. An exposure latitude of 2.6 log E can just accommodate the typical bride and groom wedding scene. An exposure latitude of at least 3.0 log E is preferred, since

this allows for a comfortable margin of error in exposure level selection by a photographer. Even larger exposure latitudes are specifically preferred, since the ability to obtain accurate image reproduction with larger exposure errors is realized. Whereas in color negative elements intended for printing, the visual attractiveness of the printed scene is often lost when gamma is exceptionally low, when color negative elements are scanned to create digital dye image records, contrast can be increased by adjustment of the electronic signal information. When the elements are scanned using a reflected beam, the beam travels through the layer units twice. This effectively doubles gamma ( $\Delta D + \Delta \log E$ ) by doubling changes in density ( $\Delta D$ ). Thus, gamma's as low as 1.0 or even 0.6 are contemplated and exposure latitudes of up to about 5.0  $\log E$  or higher are feasible. Gammas of about 0.55 are preferred. Gammas of between about 0.4 and 0.5 are especially preferred.

Instead of employing dye-forming couplers, any of the conventional incorporated dye image generating compounds employed in multicolor imaging can be alternatively incorporated in the blue, green and red recording layer units. Dye images can be produced by the selective destruction, formation or physical removal of dyes as a function of exposure.

It is also well known that preformed image dyes can be incorporated in blue, green and red recording layer units, the dyes being chosen to be initially immobile, but capable of releasing the dye chromophore in a mobile moiety as a function of entering into a redox reaction with oxidized developing agent. These compounds are commonly referred to as redox dye releasers (RDR's). By washing out the released mobile dyes, a retained dye image is created that can be scanned. It is also possible to transfer the released mobile dyes to a receiver, where they are immobilized in a mordant layer. The image-bearing receiver can then be scanned. Initially the receiver is an integral part of the color negative element. When scanning is conducted with the receiver remaining an integral part of the element, the receiver typically contains a transparent support, the dye image bearing mordant layer just beneath the support, and a white reflective layer just beneath the mordant layer. Where the receiver is peeled from the color negative element to facilitate scanning of the dye image, the receiver support can be reflective, as is commonly the choice when the dye image is intended to be viewed, or transparent, which allows transmission scanning of the dye image. RDR's as well as dye image transfer systems in which they are incorporated are described in *Research Disclosure*, Vol. 151, November 1976, Item 15162.

It is also recognized that the dye image can be provided by compounds that are initially mobile, but are rendered immobile during imagewise development. Image transfer systems utilizing imaging dyes of this type have long been used in previously disclosed dye image transfer systems. These and other image transfer systems compatible with the practice of the invention are disclosed in *Research Disclosure*, Vol. 176, December 1978, Item 17643, XXIII. Image transfer systems.

A number of modifications of color negative elements have been suggested for accommodating scanning, as illustrated by *Research Disclosure* I, Section XIV. Scan facilitating features. These systems to the extent compatible with the color negative element constructions described above are contemplated for use in the practice of this invention.

It is also contemplated that the imaging element of this invention may be used with non-conventional sensitization

schemes. For example, instead of using imaging layers sensitized to the red, green, and blue regions of the spectrum, the light-sensitive material may have one white-sensitive layer to record scene luminance, and two color-sensitive layers to record scene chrominance. Following development, the resulting image can be scanned and digitally reprocessed to reconstruct the full colors of the original scene as described in U.S. Pat. No. 5,962,205. The imaging element may also comprise a pan-sensitized emulsion with accompanying color-separation exposure. In this embodiment, the developers of the invention would give rise to a colored or neutral image which, in conjunction with the separation exposure, would enable full recovery of the original scene color values. In such an element, the image may be formed by either developed silver density, a combination of one or more conventional couplers, or "black" couplers such as resorcinol couplers. The separation exposure may be made either sequentially through appropriate filters, or simultaneously through a system of spatially discreet filter elements (commonly called a "color filter array").

The imaging element may also be a black and white image-forming material comprised, for example, of a pan-sensitized silver halide emulsion and a developer of the invention. In this embodiment, the image may be formed by developed silver density following processing, or by a coupler that generates a dye which can be used to carry the neutral image tone scale.

When conventional yellow, magenta, and cyan image dyes are formed to read out the recorded scene exposures following chemical development of conventional exposed color photographic materials, the response of the red, green, and blue color recording units of the element can be accurately discerned by examining their densities. Densitometry is the measurement of transmitted light by a sample using selected colored filters to separate the imagewise response of the RGB image dye forming units into relatively independent channels. It is common to use Status M filters to gauge the response of color negative film elements intended for optical printing, and Status A filters for color reversal films intended for direct transmission viewing. In integral densitometry, the unwanted side and tail absorptions of the imperfect image dyes leads to a small amount of channel mixing, where part of the total response of, for example, a magenta channel may come from off-peak absorptions of either the yellow or cyan image dyes records, or both, in neutral characteristic curves. Such artifacts may be negligible in the measurement of a film's spectral sensitivity. By appropriate mathematical treatment of the integral density response, these unwanted off-peak density contributions can be completely corrected providing analytical densities, where the response of a given color record is independent of the spectral contributions of the other image dyes. Analytical density determination has been summarized in the *SPSE Handbook of Photographic Science and Engineering*, W. Thomas, editor, John Wiley and Sons, New York, 1973, Section 15.3, Color Densitometry, pp. 840-848.

Image noise can be reduced, where the images are obtained by scanning exposed and processed color negative film elements to obtain a manipulatable electronic record of the image pattern, followed by reconversion of the adjusted electronic record to a viewable form. Image sharpness and colorfulness can be increased by designing layer gamma ratios to be within a narrow range while avoiding or minimizing other performance deficiencies, where the color record is placed in an electronic form prior to recreating a color image to be viewed. Whereas it is impossible to

separate image noise from the remainder of the image information, either in printing or by manipulating an electronic image record, it is possible by adjusting an electronic image record that exhibits low noise, as is provided by color negative film elements with low gamma ratios, to improve overall curve shape and sharpness characteristics in a manner that is impossible to achieve by known printing techniques. Thus, images can be recreated from electronic image records derived from such color negative elements that are superior to those similarly derived from conventional color negative elements constructed to serve optical printing applications. The excellent imaging characteristics of the described element are obtained when the gamma ratio for each of the red, green and blue color recording units is less than 1.2. In a more preferred embodiment, the red, green, and blue light sensitive color forming units each exhibit gamma ratios of less than 1.15. In an even more preferred embodiment, the red and blue light sensitive color forming units each exhibit gamma ratios of less than 1.10. In a most preferred embodiment, the red, green, and blue light sensitive color forming units each exhibit gamma ratios of less than 1.10. In all cases, it is preferred that the individual color unit(s) exhibit gamma ratios of less than 1.15, more preferred that they exhibit gamma ratios of less than 1.10 and even more preferred that they exhibit gamma ratios of less than 1.05. The gamma ratios of the layer units need not be equal. These low values of the gamma ratio are indicative of low levels of interlayer interaction, also known as interlayer interimage effects, between the layer units and are believed to account for the improved quality of the images after scanning and electronic manipulation. The apparently deleterious image characteristics that result from chemical interactions between the layer units need not be electronically suppressed during the image manipulation activity. The interactions are often difficult if not impossible to suppress properly using known electronic image manipulation schemes.

Elements having excellent light sensitivity are best employed in the practice of this invention. The elements should have a sensitivity of at least about ISO 50, preferably have a sensitivity of at least about ISO 100, and more preferably have a sensitivity of at least about ISO 200. Elements having a sensitivity of up to ISO 3200 or even higher are specifically contemplated. The speed, or sensitivity, of a color negative photographic element is inversely related to the exposure required to enable the attainment of a specified density above fog after processing. Photographic speed for a color negative element with a gamma of about 0.65 in each color record has been specifically defined by the American National Standards Institute (ANSI) as ANSI Standard Number PH 2.27-1981 (ISO (ASA Speed)) and relates specifically the average of exposure levels required to produce a density of 0.15 above the minimum density in each of the green light sensitive and least sensitive color recording unit of a color film. This definition conforms to the International Standards Organization (ISO) film speed rating. For the purposes of this application, if the color unit gammas differ from 0.65, the ASA or ISO speed is to be calculated by linearly amplifying or deamplifying the gamma vs. log E (exposure) curve to a value of 0.65 before determining the speed in the otherwise defined manner.

The present invention also contemplates the use of photographic elements in what are often referred to as single use cameras (or "film with lens" units). These cameras are sold with film preloaded in them and the entire camera is returned to a processor with the exposed film remaining inside the

camera. The one-time-use cameras employed in this invention can be any of those known in the art. These cameras can provide specific features as known in the art such as shutter means, film winding means, film advance means, waterproof housings, single or multiple lenses, lens selection means, variable aperture, focus or focal length lenses, means for monitoring lighting conditions, means for adjusting shutter times or lens characteristics based on lighting conditions or user provided instructions, and means for camera recording use conditions directly on the film. These features include, but are not limited to: providing simplified mechanisms for manually or automatically advancing film and resetting shutters as described at Skarman, U.S. Pat. No. 4,226,517; providing apparatus for automatic exposure control as described at Matterson et al, U.S. Pat. No. 4,345,835; moisture-proofing as described at Fujimura et al, U.S. Pat. No. 4,766,451; providing internal and external film casings as described at Ohmura et al, U.S. Pat. No. 4,751,536; providing means for recording use conditions on the film as described at Taniguchi et al, U.S. Pat. No. 4,780,735; providing lens fitted cameras as described at Arai, U.S. Pat. No. 4,804,987; providing film supports with superior anti-curl properties as described at Sasaki et al, U.S. Pat. No. 4,827,298; providing a viewfinder as described at Ohmura et al, U.S. Pat. No. 4,812,863; providing a lens of defined focal length and lens speed as described at Ushiro et al, U.S. Pat. No. 4,812,866; providing multiple film containers as described at Nakayama et al, U.S. Pat. No. 4,831,398 and at Ohmura et al, U.S. Pat. No. 4,833,495; providing films with improved anti-friction characteristics as described at Shiba, U.S. Pat. No. 4,866,469; providing winding mechanisms, rotating spools, or resilient sleeves as described at Mochida, U.S. Pat. No. 4,884,087; providing a film patron or cartridge removable in an axial direction as described by Takei et al at U.S. Pat. No. 4,890,130 and 5,063,400; providing an electronic flash means as described at Ohmura et al, U.S. Pat. No. 4,896,178; providing an externally operable member for effecting exposure as described at Mochida et al, U.S. Pat. No. 4,954,857; providing film support with modified sprocket holes and means for advancing said film as described at Murakami, U.S. Pat. No. 5,049,908; providing internal mirrors as described at Hara, U.S. Pat. No. 5,084,719; and providing silver halide emulsions suitable for use on tightly wound spools as described at Yagi et al, European Pat. No. Application 0,466,417 A.

While the film may be mounted in the one-time-use camera in any manner known in the art, it is especially preferred to mount the film in the one-time-use camera such that it is taken up on exposure by a thrust cartridge. Thrust cartridges are disclosed by Kataoka et al U.S. Pat. No. 5,226,613; by Zander U.S. Pat. No. 5,200,777; by Dowling et al U.S. Pat. No. 5,031,852; and by Robertson et al U.S. Pat. No. 4,834,306. Narrow bodied one-time-use cameras suitable for employing thrust cartridges in this way are described by Tobioka et al U.S. Pat. No. 5,692,221.

Cameras may contain a built-in processing capability, for example a heating element. Designs for such cameras including their use in an image capture and display system are disclosed in U.S. patent application Ser. No. 09/388,573 filed Sep. 1, 1999. The use of a one-time use camera as disclosed in said application is particularly preferred in the practice of this invention.

Photographic elements of the present invention are preferably imagewise exposed using any of the known techniques, including those described in *Research Disclosure I*, Section XVI. This typically involves exposure to light in the visible region of the spectrum, and typically such

exposure is of a live image through a lens, although exposure can also be exposure to a stored image (such as a computer stored image) by means of light emitting devices (such as light emitting diodes, CRT and the like). The photothermographic elements are also exposed by means of various forms of energy, including ultraviolet and infrared regions of the electromagnetic spectrum as well as electron beam and beta radiation, gamma ray, x-ray, alpha particle, neutron radiation and other forms of corpuscular wave-like radiant energy in either non-coherent (random phase) or coherent (in phase) forms produced by lasers. Exposures are monochromatic, orthochromatic, or panchromatic depending upon the spectral sensitization of the photographic silver halide.

The elements as discussed above may serve as origination material for some or all of the following processes: image scanning to produce an electronic rendition of the capture image, and subsequent digital processing of that rendition to manipulate, store, transmit, output, or display electronically that image.

The method of this invention may be used for photographic elements that contain any or all of the features discussed above, but are intended for thermal process systems (thermographic and photothermographic), where processing is initiated by the application of heat to the imaging element.

Photothermographic elements of the type described in *Research Disclosure* 17029 are included by reference. The photothermographic elements may be of type A or type B as disclosed in *Research Disclosure* I. Type A elements contain in reactive association a photosensitive silver halide, a reducing agent or developer, an activator, and a coating vehicle or binder. In these systems development occurs by reduction of silver ions in the photosensitive silver halide to metallic silver. Type B systems can contain all of the elements of a type A system in addition to a salt or complex of an organic compound with silver ion. In these systems, this organic complex is reduced during development to yield silver metal. The organic silver salt will be referred to as the silver donor. References describing such imaging elements include, for example, U.S. Pat. Nos. 3,457,075; 4,459,350; 4,264,725 and 4,741,992.

The photothermographic element comprises a photosensitive component that consists essentially of photographic silver halide. In the type B photothermographic material it is believed that the latent image silver from the silver halide acts as a catalyst for the described image-forming combination upon processing. In these systems, a preferred concentration of photographic silver halide is within the range of 0.01 to 100 moles of photographic silver halide per mole of silver donor in the photothermographic material.

The Type B photothermographic element comprises an oxidation-reduction image forming combination that contains an organic silver salt oxidizing agent. The organic silver salt is a silver salt which is comparatively stable to light, but aids in the formation of a silver image when heated to 80° C. or higher in the presence of an exposed photocatalyst (i.e., the photosensitive silver halide) and a reducing agent.

Suitable organic silver salts include silver salts of organic compounds having a carboxyl group. Preferred examples thereof include a silver salt of an aliphatic carboxylic acid and a silver salt of an aromatic carboxylic acid. Preferred examples of the silver salts of aliphatic carboxylic acids include silver behenate, silver stearate, silver oleate, silver laureate, silver caprate, silver myristate, silver palmitate,

silver maleate, silver fumarate, silver tartarate, silver furoate, silver linoleate, silver butyrate and silver camphorate, mixtures thereof, etc. Silver salts which are substitutable with a halogen atom or a hydroxyl group can also be effectively used. Preferred examples of the silver salts of aromatic carboxylic acid and other carboxyl group-containing compounds include silver benzoate, a silver-substituted benzoate such as silver 3,5-dihydroxybenzoate, silver o-methylbenzoate, silver m-methylbenzoate, silver p-methylbenzoate, silver 2,4-dichlorobenzoate, silver acetamidobenzoate, silver p-phenylbenzoate, etc., silver gallate, silver tannate, silver phthalate, silver terephthalate, silver salicylate, silver phenylacetate, silver pyromellitate, a silver salt of 3-carboxymethyl-4-methyl-4-thiazoline-2-thione or the like as described in U.S. Pat. No. 3,785,830, and silver salt of an aliphatic carboxylic acid containing a thioether group as described in U.S. Pat. No. 3,330,663.

Silver salts of mercapto or thione substituted compounds having a heterocyclic nucleus containing 5 or 6 ring atoms, at least one of which is nitrogen, with other ring atoms including carbon and up to two hetero-atoms selected from among oxygen, sulfur and nitrogen are specifically contemplated. Typical preferred heterocyclic nuclei include triazole, oxazole, thiazole, thiazoline, imidazoline, imidazole, diazole, pyridine and triazine. Preferred examples of these heterocyclic compounds include a silver salt of 3-mercaptop-4-phenyl-1,2,4-triazole, a silver salt of 2-mercaptopbenzimidazole, a silver salt of 2-mercaptop-5-aminothiadiazole, a silver salt of 2-(2-ethyl-glycolamido)benzothiazole, a silver salt of 5-carboxylic-1-methyl-2-phenyl-4-5 thiopyridine, a silver salt of mercaptotriazine, a silver salt of 2-mercaptopbenzoxazole, a silver salt as described in U.S. Pat. No. 4,123, 274, for example, a silver salt of 1,2,4-mercaptopthiazole derivative such as a silver salt of 3-amino-5-benzylthio-1,2,4-thiazole, a silver salt of a thione compound such as a silver salt of 3-(2-carboxyethyl)-4-methyl-4-thiazoline-2-thione as disclosed in U.S. Pat. No. 3,201,678. Examples of other useful mercapto or thione substituted compounds that do not contain a heterocyclic nucleus are illustrated by the following: a silver salt of thioglycolic acid such as a silver salt of a S-alkylthioglycolic acid (wherein the alkyl group has from 12 to 22 carbon atoms) as described in Japanese patent application 28221/73, a silver salt of a dithiocarboxylic acid such as a silver salt of dithioacetic acid, and a silver salt of thioamide.

Furthermore, a silver salt of a compound containing an imino group can be used. Preferred examples of these compounds include a silver salt of benzotriazole and a derivative thereof as described in Japanese patent publications 30270/69 and 18146/70, for example a silver salt of benzotriazole or methylbenzotriazole, a silver salt of a halogen substituted benzotriazole, such as a silver salt of 5-chlorobenzotriazole, a silver salt of 1,2,4-triazole, a silver salt of 3-amino-5-mercaptopbenzyl-1,2,4-triazole, of 1H-tetrazole as described in U.S. Pat. No. 4,220,709, a silver salt of imidazole and an imidazole derivative.

It is also found convenient to use silver half soap, of which an equimolar blend of a silver behenate with behenic acid, prepared by precipitation from aqueous solution of the sodium salt of commercial behenic acid and analyzing about 14.5 percent silver, represents a preferred example. Transparent sheet materials made on transparent film backing require a transparent coating and for this purpose the silver behenate full soap, containing not more than about 4 or 5 percent of free behenic acid and analyzing about 25.2 percent silver may be used. A method for making silver soap dispersions is well known in the art and is disclosed in

Research Disclosure October 1983 (23419) and U.S. Pat. No. 3,985,565.

Silver salts complexes may also be prepared by mixture of aqueous solutions of a silver ionic species, such as silver nitrate, and a solution of the organic ligand to be complexed with silver. The mixture process may take any convenient form, including those employed in the process of silver halide precipitation. A stabilizer may be used to avoid flocculation of the silver complex particles. The stabilizer may be any of those materials known to be useful in the photographic art, such as, but not limited to, gelatin, polyvinyl alcohol or polymeric or monomeric surfactants.

The photosensitive silver halide grains and the organic silver salt are coated so that they are in catalytic proximity during development. They can be coated in contiguous layers, but are preferably mixed prior to coating. Conventional mixing techniques are illustrated by *Research Disclosure*, Item 17029, cited above, as well as U.S. Pat. No. 3,700,458 and published Japanese patent applications Nos. 32928/75, 13224/74, 17216/75 and 42729/76.

A reducing agent in addition to the developer may be included. The reducing agent for the organic silver salt may be any material, preferably organic material, that can reduce silver ion to metallic silver. Conventional photographic developers such as 3-pyrazolidinones, hydroquinones, p-aminophenols, p-phenylenediamines and catechol are useful, but hindered phenol reducing agents are preferred. The reducing agent is preferably present in a concentration ranging from 5 to 25 percent of the photothermographic layer.

A wide range of reducing agents has been disclosed in dry silver systems including amidoximes such as phenylamidoxime, 2-thienylamidoxime and p-phenoxyphenylamidoxime, azines (e.g., 4-hydroxy-3,5-dimethoxybenzaldehydeazine); a combination of aliphatic carboxylic acid aryl hydrazides and ascorbic acid, such as 2,2'-bis(hydroxymethyl)propionylbetaphenyl hydrazide in combination with ascorbic acid; an combination of polyhydroxybenzene and hydroxylamine, a reductone and/or a hydrazine, e.g., a combination of hydroquinone and bis(ethoxyethyl)hydroxylamine, piperidinohexose reductone or formyl-4-methylphenylhydrazine, hydroxamic acids such as phenylhydroxamic acid, p-hydroxyphenyl-hydroxamic acid, and o-alaninehydroxamic acid; a combination of azines and sulfonamidophenols, e.g., phenothiazine and 2,6-dichloro-4-benzenesulfonamidophenol;  $\alpha$ -cyano-phenylacetic acid derivatives such as ethyl  $\alpha$ -cyano-2-methylphenylacetate, ethyl  $\alpha$ -cyano-phenylacetate; bis- $\alpha$ -naphthols as illustrated by 2,2'-dihydroxyl-1-binaphthyl, 6,6'-dibromo-2,2'-dihydroxy-1,1'-binaphthyl, and bis(2-hydroxy-1-naphthyl) methane; a combination of bis-o-naphthol and a 1,3-dihydroxybenzene derivative, (e.g., 2,4-dihydroxybenzophenone or 2,4-dihydroxyacetophenone); 5-pyrazolones such as 3-methyl-1-phenyl-5-pyrazolone; reductones as illustrated by dimethylaminohexose reductone, anhydrodihydroaminohexose reductone, and anhydrodihydro-piperidone-hexose reductone; sulfamidophenol reducing agents such as 2,6-dichloro-4-benzene-sulfon-amido-phenol, and p-benzenesulfonamidophenol; 2-phenylindane-1,3-dione and the like; chromans such as 2,2-dimethyl-7-t-butyl-6-hydroxychroman; 1,4-dihydropyridines such as 2,6-dimethoxy-3,5-dicarbethoxy-1,4-dihydropyridene; bisphenols, e.g., bis(2-hydroxy-3-t-butyl-5-methylphenyl)-methane; 2,2-bis(4-hydroxy-3-methylphenyl)-propane; 4,4-ethylidene-bis(2-t-butyl-6-methylphenol); and 2,2-bis(3,5-dimethyl-4-hydroxyphenyl)-propane; ascorbic acid derivatives, e.g., 1-ascorbyl-

palmitate, ascorbylstearate and unsaturated aldehydes and ketones, such as benzyl and diacetyl; pyrazolidin-3-ones; and certain indane-1,3-diones.

An optimum concentration of organic reducing agent in the photothermographic element varies depending upon such factors as the particular photothermographic element, desired image, processing conditions, the particular organic silver salt and the particular oxidizing agent.

The photothermographic element can comprise a toning agent, also known as an activator-toner or toner-accelerator. Combinations of toning agents are also useful in the photothermographic element. Examples of useful toning agents and toning agent combinations are described in, for example, *Research Disclosure*, June 1978, Item No. 17029 and U.S. Pat. No. 4,123,282. Examples of useful toning agents include, for example, phthalimide, N-hydroxyphthalimide, N-potassium-phthalimide, succinimide [too soluble], N-hydroxy-1,8-naphthalimide, phthalazine, 1-(2H)-phthalazinone, 2-acetylphthalazinone and salicylanilide.

Post-processing image stabilizers and latent image keeping stabilizers are useful in the photothermographic element. Any of the stabilizers known in the photothermographic art are useful for the described photothermographic element. Illustrative examples of useful stabilizers include photolytically active stabilizers and stabilizer precursors as described in, for example, U.S. Pat. No. 4,459,350. Other examples of useful stabilizers include azole thioethers and blocked azolinethione stabilizer precursors and carbamoyl stabilizer precursors, such as described in U.S. Pat. No. 3,877,940.

The photothermographic elements preferably contain various colloids and polymers alone or in combination as vehicles and binders and in various layers. Useful materials are hydrophilic or hydrophobic. They are transparent or translucent and include both naturally occurring substances, such as gelatin, gelatin derivatives, cellulose derivatives, polysaccharides, such as dextran, gum arabic and the like; and synthetic polymeric substances, such as water-soluble polyvinyl compounds like poly(vinylpyrrolidone) and acrylamide polymers. Other synthetic polymeric compounds that are useful include dispersed vinyl compounds such as in latex form and particularly those that increase dimensional stability of photographic elements. Effective polymers include water insoluble polymers of acrylates, such as alkylacrylates and methacrylates, acrylic acid, sulfoacrylates, and those that have cross-linking sites. Preferred high molecular weight materials and resins include poly(vinyl butyral), cellulose acetate butyrate, poly(methylmethacrylate), poly(vinylpyrrolidone), ethyl cellulose, polystyrene, poly(vinylchloride), chlorinated rubbers, polyisobutylene, butadiene-styrene copolymers, copolymers of vinyl chloride and vinyl acetate, copolymers of vinylidene chloride and vinyl acetate, poly(vinyl alcohol) and polycarbonates. When coatings are made using organic solvents, organic soluble resins may be coated by direct mixture into the coating formulations. When coating from aqueous solution, any useful organic soluble materials may be incorporated as a latex or other fine particle dispersion.

Photothermographic elements as described can contain addenda that are known to aid in formation of a useful image. The photothermographic element can contain development modifiers that function as speed increasing compounds, sensitizing dyes, hardeners, antistatic agents, plasticizers and lubricants, coating aids, brighteners, absorbing and filter dyes, such as described in *Research Disclosure*, December 1978, Item No. 17643 and *Research Disclosure*, June 1978, Item No. 17029.

The layers of the photothermographic element are coated on a support by coating procedures known in the photographic art, including dip coating, air knife coating, curtain coating or extrusion coating using hoppers. If desired, two or more layers are coated simultaneously.

A photothermographic element as described preferably comprises a thermal stabilizer to help stabilize the photothermographic element prior to exposure and processing. Such a thermal stabilizer provides improved stability of the photothermographic element during storage. Preferred thermal stabilizers are 2-bromo-2-arylsulfonylacetamides, such as 2-bromo-2-p-tolylsulfonylacetamide; 2-(tribromomethyl sulfonyl)benzothiazole; and 6-substituted-2,4-bis (tribromomethyl)-s-triazines, such as 6-methyl or 6-phenyl-2,4-bis(tribromomethyl)-s-triazine.

Imagewise exposure is preferably for a time and intensity sufficient to produce a developable latent image in the photothermographic element.

After imagewise exposure of the photothermographic element, the resulting latent image can be developed in a variety of ways. The simplest is by overall heating the element to thermal processing temperature. This overall heating merely involves heating the photothermographic element to a temperature within the range of about 90° C. to about 180° C. until a developed image is formed, such as within about 0.5 to about 60 seconds. By increasing or decreasing the thermal processing temperature a shorter or longer time of processing is useful. A preferred thermal processing temperature is within the range of about 100° C. to about 160° C. Heating means known in the photothermographic arts are useful for providing the desired processing temperature for the exposed photothermographic element. The heating means is, for example, a simple hot plate, iron, roller, heated drum, microwave heating means, heated air, vapor or the like.

It is contemplated that the design of the processor for the hotothermographic element be linked to the design of the cassette or cartridge used for storage and use of the element. Further, data stored on the film or cartridge may be used to modify processing conditions or scanning of the element. Methods for accomplishing these steps in the imaging system are disclosed in commonly assigned, co-pending U.S. patent applications Ser. Nos. 09/206586, 09/206,612, and 09/206,583 filed Dec. 7, 1998. The use of an apparatus whereby the processor can be used to write information onto the element, information which can be used to adjust processing, scanning, and image display is also envisaged. This system is disclosed in U.S. patent applications Ser. Nos. 09/206,914 filed Dec. 7, 1998 and 09/333,092 filed Jun. 15, 1999.

Thermal processing is preferably carried out under ambient conditions of pressure and humidity. Conditions outside of normal atmospheric pressure and humidity are useful.

The components of the photothermographic element can be in any location in the element that provides the desired image. If desired, one or more of the components can be in one or more layers of the element. For example, in some cases, it is desirable to include certain percentages of the reducing agent, toner, stabilizer and/or other addenda in the overcoat layer over the photothermographic image recording layer of the element. This, in some cases, reduces migration of certain addenda in the layers of the element.

In accordance with one aspect of this invention the fixer sheet used in the invention is incorporated in or used in combination with a thermographic element. In thermographic elements an image is formed by imagewise heating

the element. Such elements are described in, for example, *Research Disclosure*, June 1978, Item No. 17029 and U.S. Pat. Nos. 3,080,254, 3,457,075 and 3,933,508. The thermal energy source and means for imaging can be any imagewise thermal exposure source and means that are known in the thermographic imaging art. The thermographic imaging means can be, for example, an infrared heating means, laser, or microwave heating means.

In accordance with another aspect of this invention, the fixer sheet used in the invention is incorporated in or used in combination with a photographic element in the context of low volume aqueous processing in combination with the application of heat. Low volume processing is defined as processing where the volume of applied developer solution is between about 0.1 to about 10 times, preferably about 0.5 to about 10 times, the volume of solution required to swell the photographic element. This processing may take place by a combination of solution application, external layer lamination, and heating. The low volume processing system may contain any of the elements described above for Type I: Photothermographic systems. In addition, it is specifically contemplated that any components described in the preceding sections that are not necessary for the formation or stability of latent image in the origination film element can be removed from the film element altogether and contacted at any time after exposure for the purpose of carrying out photographic processing, using the methods described below. According to this process, the photographic element may receive some or all of the following treatments:

- (I) Application of a solution directly to the film by any means, including spray, inkjet, coating and gravure process.
- (II) Soaking of the film in a reservoir containing a processing solution. This process may also take the form of dipping or passing an element through a small cartridge.
- (III) Lamination of an auxiliary processing element e.g. a fixer sheet used in the invention to the imaging element. The laminate may have the purpose of providing processing chemistry, removing spent chemistry, or transferring image information from the latent image recording film element. The transferred image may result from a dye, dye precursor, or silver containing compound being transferred in a image-wise manner to the auxiliary processing element.
- (IV) Heating of the element by any convenient means, including a simple hot plate, iron, roller, heated drum, microwave heating means, heated air, vapor, or the like. Heating may be accomplished before, during, after, or throughout any of the preceding treatments I-III. Heating may cause processing temperatures ranging from room temperature to 100° C.

In accordance with another aspect of this invention the fixer sheet used in the invention is incorporated in or used in combination with a conventional photographic element.

Conventional photographic elements can be processed in any of a number of well-known photographic processes utilizing any of a number of well-known conventional photographic processing solutions, described, for example, in *Research Disclosure I*, or in T. H. James, editor, *The Theory of the Photographic Process*, 4th Edition, Macmillan, New York, 1977. The development process may take place for any length of time and any process temperature that is suitable to render an acceptable image. In the case of processing a negative working color element, the element is treated with a color developer (that is one which will form

the colored image dyes with the color couplers), and then optionally with an oxidizer to oxidize metallic silver to silver salt. In the case of processing a reversal color element, the element is first treated with a black and white developer (that is, a developer which does not form colored dyes with the coupler compounds) followed by a treatment to fog silver halide (usually chemical fogging or light fogging), followed by treatment with a color developer. Preferred color developing agents are p-phenylenediamines. Especially preferred are:

- 4-amino N,N-diethylaniline hydrochloride,
- 4-amino-3-methyl-N,N-diethylaniline hydrochloride,
- 4-amino-3-methyl-N-ethyl-N-(2-(methanesulfonamido)ethylaniline sesquisulfate hydrate,
- 4-amino-3-methyl-N-ethyl-N-(2-hydroxyethyl)aniline sulfate,
- 4-amino-3-?--(methanesulfonamido)ethyl-N,N-diethylaniline hydrochloride and
- 4-amino-N-ethyl-N-(2-methoxyethyl)-m-toluidine di-p-toluene sulfonic acid.

Dye images can be formed or amplified by processes which employ in combination with a dye-image-generating reducing agent an inert transition metal-ion complex oxidizing agent, as illustrated by Bissonette U.S. Pat. Nos. 3,748,138, 3,826,652, 3,862,842 and 3,989,526 and Travis U.S. Pat. No. 3,765,891, and/or a peroxide oxidizing agent as illustrated by Matejec U.S. Pat. No. 3,674,490, *Research Disclosure*, Vol. 116, December, 1973, Item 11660, and Bissonette *Research Disclosure*, Vol. 148, August, 1976, Items 14836, 14846 and 14847. The photographic elements can be particularly adapted to form dye images by such processes as illustrated by Dunn et al U.S. Pat. No. 3,822,129, Bissonette U.S. Pat. Nos. 3,834,907 and 3,902,905, Bissonette et al U.S. Pat. No. 3,847,619, Mowrey U.S. Pat. No. 3,904,413, Hirai et al U.S. Pat. No. 4,880,725, Iwano U.S. Pat. No. 4,954,425, Marsden et al U.S. Pat. No. 4,983,504, Evans et al U.S. Pat. No. 5,246,822, Twist U.S. Pat. No. 5,324,624, Fyson EPO 0 487 616, Tannahill et al WO 90/13059, Marsden et al WO 90/13061, Grimsey et al WO 91/16666, Fyson WO 91/17479, Marsden et al WO 92/01972, Tannahill WO 92/05471, Henson WO 92/07299, Twist WO 93/01524 and WO 93/11460 and Wingender et al German OLS 4,211,460.

Development may be followed by bleaching to oxidize metallic silver to a silver salt, washing and drying.

Once yellow, magenta, and cyan dye image records have been formed in photographic elements which have been processed in accordance with the invention, conventional techniques can be employed for retrieving the image information for each color record and manipulating the record for subsequent creation of a color balanced viewable image. For example, it is possible to scan the photographic element successively within the blue, green, and red regions of the spectrum or to incorporate blue, green, and red light within a single scanning beam that is divided and passed through blue, green, and red filters to form separate scanning beams for each color record. A simple technique is to scan the photographic element point-by-point along a series of laterally offset parallel scan paths. The intensity of light passing through the element at a scanning point is noted by a sensor which converts radiation received into an electrical signal. Most generally this electronic signal is further manipulated to form a useful electronic record of the image. For example, the electrical signal can be passed through an analog-to-digital converter and sent to a digital computer together with location information required for pixel (point)

location within the image. In another embodiment, this electronic signal is encoded with calorimetric or tonal information to form an electronic record that is suitable to allow reconstruction of the image into viewable forms such as computer monitor displayed images, television images, printed images, and so forth.

It is generally found that improved scanned image quality can be obtained by the use of scanners that employ diffuse illumination optics. Any technique known in the art for producing diffuse illumination can be used. Preferred systems include reflective systems, that employ a diffusing cavity whose interior walls are specifically designed to produce a high degree of diffuse reflection, and transmissive systems, where diffusion of a beam of specular light is accomplished by the use of an optical element placed in the beam that serves to scatter light. Such elements can be either glass or plastic that either incorporate a component that produces the desired scattering, or have been given a surface treatment to promote the desired scattering.

One of the challenges encountered in producing images from information extracted by scanning is that the number of pixels of information available for viewing is only a fraction of that available from a comparable classical photographic print. It is, therefore, even more important in scan imaging to maximize the quality of the image information available. Enhancing image sharpness and minimizing the impact of aberrant pixel signals (i.e., noise) are common approaches to enhancing image quality. A conventional technique for minimizing the impact of aberrant pixel signals is to adjust each pixel density reading to a weighted average value by factoring in readings from adjacent pixels, closer adjacent pixels being weighted more heavily.

The elements of the invention can have density calibration patches derived from one or more patch areas on a portion of unexposed photographic recording material that was subjected to reference exposures, as described by Wheeler et al U.S. Pat. No. 5,649,260, Koeng et al U.S. Pat. No. 5,563,717, and by Cosgrove et al U.S. Pat. No. 5,644,647.

Illustrative systems of scan signal manipulation, including techniques for maximizing the quality of image records, are disclosed by Bayer U.S. Pat. No. 4,553,156; Urabe et al U.S. Pat. No. 4,591,923; Sasaki et al U.S. Pat. No. 631,578; Alkofer U.S. Pat. No. 4,654,722; Yamada et al U.S. Pat. No. 4,670,793; Ieles U.S. Pat. Nos. 4,694,342 and 4,962,542; Powell U.S. Pat. No. 4,805,031; Mayne et al U.S. Pat. No. 4,829,370; Abdulwahab U.S. Pat. No. 4,839,721; Matsunawa et al U.S. Pat. Nos. 4,841,361 and 4,937,662; Mizukoshi et al U.S. Pat. No. 4,891,713; Petilli U.S. Pat. No. 4,912,569; Sullivan et al U.S. Pat. Nos. 4,920,501 and 5,070,413; Kimoto et al Pat. No. 4,972,256; Kaplan U.S. Pat. No. 4,977,521; Sakai U.S. Pat. No. 4,979,027; Ng U.S. Pat. No. 5,003,494; Katayama et al U.S. Pat. No. 5,008,950; Kimura et al U.S. Pat. No. 5,065,255; Osamu et al U.S. Pat. No. 5,051,842; Lee et al U.S. Pat. No. 5,012,333; Bowers et al U.S. Pat. No. 5,107,346; Telle U.S. Pat. No. 5,105,266; MacDonald et al U.S. Pat. No. 5,105,469; and Kwon et al U.S. Pat. No. 5,081,692. Techniques for color balance adjustments during scanning are disclosed by Moore et al U.S. Pat. No. 5,049,984 and Davis U.S. Pat. No. 5,541,645.

The digital color records once acquired are in most instances adjusted to produce a pleasingly color balanced image for viewing and to preserve the color fidelity of the image bearing signals through various transformations or renderings for outputting, either on a video monitor or when printed as a conventional color print. Preferred techniques for transforming image bearing signals after scanning are disclosed by Giorgianni et al U.S. Pat. No. 5,267,030, the

disclosures of which are herein incorporated by reference. Further illustrations of the capability of those skilled in the art to manage color digital image information are provided by Giorgianni and Madden *Digital Color Management*, Addison-Wesley, 1998.

FIG. 1 shows, in block diagram form, the manner in which the image information provided by the color negative elements is contemplated to be used. An image scanner 2 is used to scan by transmission an imagewise exposed and photographically processed color negative element 1 according to the invention. The scanning beam is most conveniently a beam of white light that is split after passage through the layer units and passed through filters to create separate image records-red recording layer unit image record (R), green recording layer unit image record (G), and blue recording layer unit image record (B). Instead of splitting the beam, blue, green, and red filters can be sequentially caused to intersect the beam at each pixel location. In still another scanning variation, separate blue, green, and red light beams, as produced by a collection of light emitting diodes, can be directed at each pixel location. As the element 1 is scanned pixel-by-pixel using an array detector, such as an array charge-coupled device (CCD), or line-by-line using a linear array detector, such as a linear array CCD, a sequence of R, G, and B picture element signals are generated that can be correlated with spatial location information provided from the scanner. Signal intensity and location information is fed to a workstation 4, and the information is transformed into an electronic form R', G', and B', which can be stored in any convenient storage device 5.

In motion imaging industries, a common approach is to transfer the color negative film information into a video signal using a telecine transfer device. Two types of telecine transfer devices are most common: (1) a flying spot scanner using photomultiplier tube detectors or (2) CCD's as sensors. These devices transform the scanning beam that has passed through the color negative film at each pixel location into a voltage. The signal processing then inverts the electrical signal in order to render a positive image. The signal is then amplified and modulated and fed into a cathode ray tube monitor to display the image or recorded onto magnetic tape for storage. Although both analog and digital image signal manipulations are contemplated, it is preferred to place the signal in a digital form for manipulation, since the overwhelming majority of computers are now digital and this facilitates use with common computer peripherals, such as magnetic tape, a magnetic disk, or an optical disk.

A video monitor 6, which receives the digital image information modified for its requirements, indicated by R'', G'', and B'', allows viewing of the image information received by the workstation. Instead of relying on a cathode ray tube of a video monitor, a liquid crystal display panel or any other convenient electronic image viewing device can be substituted. The video monitor typically relies upon a picture control apparatus 3, which can include a keyboard and cursor, enabling the workstation operator to provide image manipulation commands for modifying the video image displayed and any image to be recreated from the digital image information.

Any modifications of the image can be viewed as they are being introduced on the video display 6 and stored in the storage device 5. The modified image information R'', G'', and B'' can be sent to an output device 7 to produce a recreated image for viewing. The output device can be any convenient conventional element writer, such as a thermal dye transfer, inkjet, electrostatic, electrophotographic,

electrostatic, thermal dye sublimation or other type of printer. CRT or LED printing to sensitized photographic paper is also contemplated. The output device can be used to control the exposure of a conventional silver halide color paper. The output device creates an output medium 8 that bears the recreated image for viewing. It is the image in the output medium that is ultimately viewed and judged by the end user for noise (granularity), sharpness, contrast, and color balance. The image on a video display may also ultimately be viewed and judged by the end user for noise, sharpness, tone scale, color balance, and color reproduction, as in the case of images transmitted between parties on the World Wide Web of the Internet computer network.

Using an arrangement of the type shown in FIG. 1, the images contained in color negative elements in accordance with the invention are converted to digital form, manipulated, and recreated in a viewable form. Color negative recording materials according to the invention can be used with any of the suitable methods described in U.S. Pat. No. 5,257,030. In one preferred embodiment, Giorgianni et al provides for a method and means to convert the R, G, and B image-bearing signals from a transmission scanner to an image manipulation and/or storage metric which corresponds to the trichromatic signals of a reference image-producing device such as a film or paper writer, thermal printer, video display, etc. The metric values correspond to those which would be required to appropriately reproduce the color image on that device. For example, if the reference image producing device was chosen to be a specific video display, and the intermediary image data metric was chosen to be the R', G', and B' intensity modulating signals (code values) for that reference video display, then for an input film, the R, G, and B image-bearing signals from a scanner would be transformed to the R', G', and B' code values corresponding to those which would be required to appropriately reproduce the input image on the reference video display. A data-set is generated from which the mathematical transformations to convert R, G, and B image-bearing signals to the aforementioned code values are derived. Exposure patterns, chosen to adequately sample and cover the useful exposure range of the film being calibrated, are created by exposing a pattern generator and are fed to an exposing apparatus. The exposing apparatus produces trichromatic exposures on film to create test images consisting of approximately 150 color patches. Test images may be created using a variety of methods appropriate for the application. These methods include: using exposing apparatus such as a sensitometer, using the output device of a color imaging apparatus, recording images of test objects of known reflectances illuminated by known light sources, or calculating trichromatic exposure values using methods known in the photographic art. If input films of different speeds are used, the overall red, green, and blue exposures must be properly adjusted for each film in order to compensate for the relative speed differences among the films. Each film thus receives equivalent exposures, appropriate for its red, green, and blue speeds. The exposed film is processed chemically. Film color patches are read by transmission scanner which produces R, G, and B image-bearing signals corresponding each color patch. Signal-value patterns of code value pattern generator produces RGB intensity-modulating signals which are fed to the reference video display. The R', G', and B' code values for each test color are adjusted such that a color matching apparatus, which may correspond to an instrument or a human observer, indicates that the video display test colors match the positive film test colors or the colors of a printed negative. A transform

apparatus creates a transform relating the R, G, and B image-bearing signal values for the film's test colors to the R', G', and B' code values of the corresponding test colors.

The mathematical operations required to transform R, G, and B image-bearing signals to the intermediary data may consist of a sequence of matrix operations and look-up tables (LUT's).

Referring to FIG. 2, in a preferred embodiment, input image-bearing signals R, G, and B are transformed to intermediary data values corresponding to the R', G', and B' output image-bearing signals required to appropriately reproduce the color image on the reference output device as follows:

- (1) The R, G, and B image-bearing signals, which correspond to the measured transmittances of the film, are converted to corresponding densities in the computer used to receive and store the signals from a film scanner by means of 1-dimensional look-up table LUT 1.
- (2) The densities from step (1) are then transformed using matrix 1 derived from a transform apparatus to create intermediary image-bearing signals.
- (3) The densities of step (2) are optionally modified with a 1-dimensional look-up table LUT 2 derived such that the neutral scale densities of the input film are transformed to the neutral scale densities of the reference.
- (4) The densities of step (3) are transformed through a 1-dimensional look-up table LUT 3 to create corresponding R', G', and B' output image-bearing signals for the reference output device.

It will be understood that individual look-up tables are typically provided for each input color. In one embodiment, three 1-dimensional look-up tables can be employed, one for each of a red, green, and blue color record. In another embodiment, a multi-dimensional look-up table can be employed as described by D'Errico at U.S. Pat. No. 4,941,039. It will be appreciated that the output image-bearing signals for the reference output device of step 4 above may be in the form of device-dependent code values or the output image-bearing signals may require further adjustment to become device specific code values. Such adjustment may be accomplished by further matrix transformation or 1-dimensional look-up table transformation, or a combination of such transformations to properly prepare the output image-bearing signals for any of the steps of transmitting, storing, printing, or displaying them using the specified device.

In a second preferred embodiment the R, G, and B image-bearing signals from a transmission scanner are converted to an image manipulation and/or storage metric which corresponds to a measurement or description of a single reference image-recording device and/or medium and in which the metric values for all input media correspond to the trichromatic values which would have been formed by the reference device or medium had it captured the original scene under the same conditions under which the input media captured that scene. For example, if the reference image recording medium was chosen to be a specific color negative film, and the intermediary image data metric was chosen to be the measured RGB densities of that reference film, then for an input color negative film according to the invention, the R, G, and B image-bearing signals from a scanner would be transformed to the R', G', and B' density values corresponding to those of an image which would have been formed by the reference color negative film had it been exposed under the same conditions under which the color negative recording material according to the invention was exposed.

Exposure patterns, chosen to adequately sample and cover the useful exposure range of the film being calibrated, are created by exposing a pattern generator and are fed to an exposing apparatus. The exposing apparatus produces trichromatic exposures on film to create test images consisting of approximately 150 color patches. Test images may be created using a variety of methods appropriate for the application. These methods include: using exposing apparatus such as a sensitometer, using the output device of a color imaging apparatus, recording images of test objects of known reflectances illuminated by known light sources, or calculating trichromatic exposure values using methods known in the photographic art. If input films of different speeds are used, the overall red, green, and blue exposures must be properly adjusted for each film in order to compensate for the relative speed differences among the films. Each film thus receives equivalent exposures, appropriate for its red, green, and blue speeds. The exposed film is processed chemically. Film color patches are read by a transmission scanner which produces R, G, and B image-bearing signals corresponding each color patch and by a transmission densitometer which produces R', G', and B' density values corresponding to each patch. A transform apparatus creates a transform relating the R, G, and B image-bearing signal values for the film's test colors to the measured R', G', and B' densities of the corresponding test colors of the reference color negative film. In another preferred variation, if the reference image recording medium was chosen to be a specific color negative film, and the intermediary image data metric was chosen to be the predetermined R', G', and B' intermediary densities of step 2 of that reference film, then for an input color negative film according to the invention, the R, G, and B image-bearing signals from a scanner would be transformed to the R', G', and B' intermediary density values corresponding to those of an image which would have been formed by the reference color negative film had it been exposed under the same conditions under which the color negative recording material according to the invention was exposed.

Thus, each input film calibrated according to the present method would yield, insofar as possible, identical intermediary data values corresponding to the R', G', and B' code values required to appropriately reproduce the color image which would have been formed by the reference color negative film on the reference output device. Uncalibrated films may also be used with transformations derived for similar types of films, and the results would be similar to those described.

The mathematical operations required to transform R, G, and B image-bearing signals to the intermediary data metric of this preferred embodiment may consist of a sequence of matrix operations and 1-dimensional LUTs. Three tables are typically provided for the three input colors. It is appreciated that such transformations can also be accomplished in other embodiments by employing a single mathematical operation or a combination of mathematical operations in the computational steps produced by the host computer including, but not limited to, matrix algebra, algebraic expressions dependent on one or more of the image-bearing signals, and n-dimensional LUTs. In one embodiment, matrix 1 of step 2 is a 3x3 matrix. In a more preferred embodiment, matrix 1 of step 2 is a 3x10 matrix. In a preferred embodiment, the 1-dimensional LUT 3 in step 4 transforms the intermediary image-bearing signals according to a color photographic paper characteristic curve, thereby reproducing normal color print image tone scale. In another preferred embodiment, LUT 3 of step 4 transforms the intermediary image-bearing

signals according to a modified viewing tone scale that is more pleasing, such as possessing lower image contrast.

Due to the complexity of these transformations, it should be noted that the transformation from R, G, and B to R', G', and B' may often be better accomplished by a 3-dimensional LUT. Such 3-dimensional LUTs may be developed according to the teachings J. D'Errico in U.S. Pat. No. 4,941,039.

It is to be appreciated that while the images are in electronic form, the image processing is not limited to the specific manipulations described above. While the image is in this form, additional image manipulation may be used including, but not limited to, standard scene balance algorithms (to determine corrections for density and color balance based on the densities of one or more areas within the negative), tone scale manipulations to amplify film under-exposure gamma, non-adaptive or adaptive sharpening via convolution or unsharp masking, red-eye reduction, and non-adaptive or adaptive grain-suppression. Moreover, the image may be artistically manipulated, zoomed, cropped, and combined with additional images or other manipulations known in the art. Once the image has been corrected and any additional image processing and manipulation has occurred, the image may be electronically transmitted to a remote location or locally written to a variety of output devices including, but not limited to, silver halide film or paper writers, thermal printers, electrophotographic printers, ink-jet printers, display monitors, CD disks, optical and magnetic electronic signal storage devices, and other types of storage and display devices as known in the art.

In yet another embodiment, the luminance and chrominance sensitization and image extraction article and method described by Arakawa et al in U.S. Pat. No. 5,962,205 can be employed.

The invention is further illustrated by way of example as follows.

#### EXAMPLE 1

Equal volumes of imidazole and ethyl cellulose powders were mixed together and melted on a steam bath which provided a temperature of 100° C. A clear, viscous solution formed, which was coated on a glass microscope slide and allowed to cool. It set to form a white opaque layer. A piece of Kodacolor Royal Gold 400 film was pressed into contact with the coated layer and the assembly heated on the steam bath. After a few seconds, it was seen that the emulsion layer had become transparent, and it remained transparent on cooling.

#### EXAMPLE 2

A thermal fixing sheet was prepared by dissolving 2 g of imidazole and 1 g of ethyl cellulose in 4 g of acetone, and coating the resultant solution onto polyethylene terephthalate film support by means of a coating knife set at a gap of 150 micrometres above the film support. The coated layer went white and opaque on drying, and the total coated laydown was found to be approximately 75 g /m<sup>2</sup> by weight, corresponding to 50 g /m<sup>2</sup> of imidazole and 25 g /m<sup>2</sup> of ethyl cellulose.

A piece of Kodacolor Royal Gold 400 film was exposed to a coloured test target by contact. It was developed in Kodak Flexicolor C41 developer for 3.25 minutes at 38° C., put in an acid stop bath for 30s, then washed in running water and briefly rinsed in the stop bath before drying. The dry film was seen to bear a coloured image, but it was opaque by reason of the silver halide emulsions retained in it.

The dry film was put into face to face contact with the thermal fixing sheet and the assembly held onto a curved aluminium block maintained at a temperature of 100° C. After approximately 15s it was seen that the film had become transparent, and retained the coloured image.

The laminated assembly was then scanned in a Kodak DLS film scanner and the output file manipulated with Photoshop software. Colour saturation was increased and brightness and colour balance adjusted to give a brightly coloured and sharp image of the test target.

#### EXAMPLE 3

A piece of Kodacolor Royal Gold 400 film was exposed to a coloured test target by contact. In darkroom conditions, it was soaked in Kodak Flexicolor C41 developer for 30s at 20° C. and all surplus solution blotted off. It was held against a curved aluminium block maintained at a temperature of 100° C. for 20s, to allow development to occur, and to dry off the water.

A piece of the thermal fixing sheet of Example 2 was then held in face-to-face contact with the film, still in contact with the curved aluminium block. It was removed after 20s and examined. A coloured image of the test target was seen against a clear background.

#### EXAMPLE 4

A small sample of the substance under test was placed on a glass slide maintained at 140° C. If it melted, a small piece of film (containing silver bromoiodide emulsions at 4.5 g/m<sup>2</sup> of silver) was placed emulsion down on the molten sample and the approximate time for the film to be rendered clear was observed. If there was no significant clearing after 1 minute it was recorded as having no clearing effect. (The best compound, imidazole, rendered the film completely clear in less than 5s).

If the substance did not melt, a small quantity of anthranilamide (m.pt. 113° C.) was added to co-melt the test substance, then the test continued as above.

The following compounds were found to have a clearing effect:

- imidazole
- 2-methyl imidazole
- 4-methyl imidazole
- 1,2-dimethyl imidazole
- benzimidazole (in presence of anthranilamide)—v. slowly
- 1,2,4-triazole
- 4-amino-1,2,4-triazole (in presence of anthranilamide)—v. slowly
- 3-amino- 1,2,4-triazole (not completely cleared, but substantially)
- pyrazole (slowly)
- sodium thiocyanate dihydrate
- ammonium thiocyanate (in presence of anthranilamide)
- 1,2,4-triazole-3-thiol (in presence of anthranilamide)
- 1-(hydroxyethyl)-tetrahydrotriazine-4-thiol (in presence of anthranilamide)
- (slowly and partially)
- thiourea (in presence of anthranilamide) (partially)

#### EXAMPLE 5

The following components are used in the example. Also included is a list of all of the chemical structures.

### Silver Salt Dispersion SS-1:

A stirred reaction vessel was charged with 431 g of lime processed gelatin and 6569 g of distilled water. A solution containing 214 g of benzotriazole, 2150 g of distilled water, and 790 g of 2.5 molar sodium hydroxide was prepared (Solution B). The mixture in the reaction vessel was adjusted to a pAg of 7.25 and a pH of 8.00 by additions of Solution B, nitric acid, and sodium hydroxide as needed.

A 41 solution of 0.54 molar silver nitrate was added to the kettle at 250 cc/minute, and the pAg was maintained at 7.25 by a simultaneous addition of solution B. This process was continued until the silver nitrate solution was exhausted, at which point the mixture was concentrated by ultrafiltration. The resulting silver salt dispersion contained fine particles of silver benzotriazole.

## Silver Salt Dispersion SS-2:

A stirred reaction vessel was charged with 431 g of lime processed gelatin and 6569 g of distilled water. A solution containing 320 g of 1-phenyl-5-mercaptopetrazole, 2044 g of distilled water, and 790 g of 2.5 molar sodium hydroxide was prepared (Solution B). The mixture in the reaction vessel was adjusted to a pAg of 7.25 and a pH of 8.00 by additions of Solution B, nitric acid, and sodium hydroxide as needed.

A 41 solution of 0.54 molar silver nitrate was added to the kettle at 250 cc/minute, and the pAg was maintained at 7.25 by a simultaneous addition of solution B. This process was continued until the silver nitrate solution was exhausted, at which point the mixture was concentrated by ultrafiltration. The resulting silver salt dispersion contained fine particles of the silver salt of 1-phenyl-5-mercaptotetrazole.

## Silver Halide Emulsions;

The emulsions employed in this example are all silver iodobromide tabular grains precipitated by conventional

means as known in the art. Table 1 below lists the various emulsions, along with their iodide content (the remainder assumed to be bromide), their dimensions, and the sensitizing dyes used to impart spectral sensitivity. All of these emulsions have been given chemical sensitizations as known in the art to produce optimum sensitivity.

TABLE 1

| Emul-sion | Spectral sensitiv-ity | Iodide content (%) | Diameter ( $\mu\text{m}$ ) | Thickness ( $\mu\text{m}$ ) | Dyes        |
|-----------|-----------------------|--------------------|----------------------------|-----------------------------|-------------|
| EY-3      | yellow                | 2                  | 1.23                       | 0.125                       | SY-1        |
| EY-4      | yellow                | 2                  | 0.45                       | 0.061                       | SY-1        |
| EY-5      | yellow                | 2                  | 0.653                      | 0.093                       | SY-1        |
| EM-3      | magenta               | 2                  | 1.23                       | 0.125                       | SM-1 + SM-3 |
| EM-4      | magenta               | 2                  | 0.45                       | 0.061                       | SM-1 + SM-3 |
| EM-5      | magenta               | 2                  | 0.653                      | 0.093                       | SM-1 + SM-3 |
| EC-3      | cyan                  | 2                  | 1.23                       | 0.125                       | SC-1 + SC-2 |
| EC-4      | cyan                  | 2                  | 0.45                       | 0.061                       | SC-1 + SC-2 |
| EC-5      | cyan                  | 2                  | 0.653                      | 0.093                       | SC-1 + SC-2 |

### Coupler Dispersion CDM-2:

A coupler dispersion was prepared by conventional means containing coupler M-2 without any additional permanent solvents.

### Coupler Dispersion CDC-1:

An oil based coupler dispersion was prepared by conventional means containing coupler C-1 and dibutyl phthalate at a weight ratio of 1:2.

### Coupler Dispersion CDY-1:

An oil based coupler dispersion was prepared by conventional means containing coupler Y-1 (381 AQF) and dibutyl phthalate at a weight ratio of 1:0.5.

M-2



-continued

C-1

Y-1



SI-1

SY-2



SM-1

SM-3



-continued  
SC-1

SC-2



Hardener-2



D-28

A heat developable colour film, having the following structure was prepared:

|               |                                                                       |
|---------------|-----------------------------------------------------------------------|
| Overcoat      | 1.1 g/m <sup>2</sup> Gelatin                                          |
|               | 0.32 g/m <sup>2</sup> Hardener-2                                      |
| Fast Yellow   | 0.54 g/m <sup>2</sup> AgBrI from emulsion EY-3                        |
|               | 0.17 g/m <sup>2</sup> silver benzotriazole from SS-1                  |
|               | 0.17 g/m <sup>2</sup> silver-1-phenyl-5-mercaptop tetrazole from SS-2 |
|               | 0.29 g/m <sup>2</sup> coupler Y-1 from dispersion CDY-1               |
|               | 0.46 g/m <sup>2</sup> Developer D-28                                  |
|               | 0.46 g/m <sup>2</sup> Salicylanilide                                  |
|               | 2.3 g/m <sup>2</sup> Gelatin                                          |
| Slow Yellow   | 0.27 g/m <sup>2</sup> AgBrI from emulsion EY-4                        |
|               | 0.16 g/m <sup>2</sup> AgBrI from emulsion EY-5                        |
|               | 0.15 g/m <sup>2</sup> silver benzotriazole from SS-1                  |
|               | 0.15 g/m <sup>2</sup> silver-1-phenyl-5-mercaptop tetrazole from SS-2 |
|               | 0.25 g/m <sup>2</sup> coupler Y-1 from dispersion CDY-1               |
|               | 0.40 g/m <sup>2</sup> Developer D-28                                  |
|               | 0.40 g/m <sup>2</sup> Salicylanilide                                  |
|               | 2.0 g/m <sup>2</sup> Gelatin                                          |
| Yellow Filter | 0.08 g/m <sup>2</sup> SY-2                                            |
| Fast Magenta  | 1.07 g/m <sup>2</sup> Gelatin                                         |
|               | 0.54 g/m <sup>2</sup> AgBrI from emulsion EM-3                        |
|               | 0.17 g/m <sup>2</sup> silver benzotriazole from SS-1                  |
|               | 0.17 g/m <sup>2</sup> silver-1-phenyl-5-mercaptop tetrazole from SS-2 |
|               | 0.29 g/m <sup>2</sup> coupler M-2 from dispersion CDM-2               |
|               | 0.46 g/m <sup>2</sup> Developer D-28                                  |
|               | 0.46 g/m <sup>2</sup> Salicylanilide                                  |
|               | 2.3 g/m <sup>2</sup> Gelatin                                          |
| Slow Yellow   | 0.27 g/m <sup>2</sup> AgBrI from emulsion EM-4                        |
|               | 0.16 g/m <sup>2</sup> AgBrI from emulsion EM-5                        |
|               | 0.15 g/m <sup>2</sup> silver benzotriazole from SS-1                  |
|               | 0.15 g/m <sup>2</sup> silver-1-phenyl-5-mercaptop tetrazole from SS-2 |
|               | 0.25 g/m <sup>2</sup> coupler M-2 from dispersion CDM-2               |
|               | 0.40 g/m <sup>2</sup> Developer D-28                                  |
|               | 0.40 g/m <sup>2</sup> Salicylanilide                                  |
|               | 2.0 g/m <sup>2</sup> Gelatin                                          |
| Interlayer    | 1.07 g/m <sup>2</sup> Gelatin                                         |

35

-continued

|                    |                                                                       |
|--------------------|-----------------------------------------------------------------------|
| Fast Cyan          | 0.54 g/m <sup>2</sup> AgBrI from emulsion EC-3                        |
|                    | 0.17 g/m <sup>2</sup> silver benzotriazole from SS-1                  |
|                    | 0.17 g/m <sup>2</sup> silver-1-phenyl-5-mercaptop tetrazole from SS-2 |
|                    | 0.29 g/m <sup>2</sup> coupler C-1 from dispersion CDC-1               |
|                    | 0.46 g/m <sup>2</sup> Developer D-28                                  |
|                    | 0.46 g/m <sup>2</sup> Salicylanilide                                  |
|                    | 2.3 g/m <sup>2</sup> Gelatin                                          |
| Slow Cyan          | 0.27 g/m <sup>2</sup> AgBrI from emulsion EC-4                        |
|                    | 0.16 g/m <sup>2</sup> AgBrI from emulsion EC-5                        |
|                    | 0.15 g/m <sup>2</sup> silver benzotriazole from SS-1                  |
|                    | 0.15 g/m <sup>2</sup> silver-1-phenyl-5-mercaptop tetrazole from SS-2 |
|                    | 0.25 g/m <sup>2</sup> coupler C-1 from dispersion CDC-1               |
|                    | 0.40 g/m <sup>2</sup> Developer D-28                                  |
|                    | 0.40 g/m <sup>2</sup> Salicylanilide                                  |
|                    | 2.0 g/m <sup>2</sup> Gelatin                                          |
| Antihalation Layer | 0.05 g/m <sup>2</sup> Carbon                                          |
| Support            | 1.6 g/m <sup>2</sup> Gelatin                                          |
|                    | Polyethylene terephthalate support (7 mil thickness)                  |

55 A thermal fixing sheet was prepared by dissolving 1.5 g of imidazole, 1 g of cellulose acetate butyrate, 0.1 g of succinic acid and 0.2 g of 1,2,4-triazole-3-thiol in 3 g of acetone and 1 g of methanol, and coating the resultant solution onto polyethylene terephthalate film support by means of a coating knife set at a gap of 150 micrometres above the film support. This gave a coating which had approximately 40 g per square metre of imidazole and 27 g per square metre of cellulose acetate butyrate. (The cellulose acetate butyrate was grade EAB 272 from the Eastman Chemical Products Corporation).

60 The heat developable colour film was exposed to a coloured test target by contact. It was developed by heating 65 at 145° C. for 25s. It was then placed in face-to-face contact with the thermal fixing sheet and the assembly passed twice through a heat lamination machine ("Esselte", model PLA4)

**35**

with the temperature set to 120° C. Two passes through the machine corresponded to a heating time of approximately 15s. The film was seen to have cleared and become non-scattering in the areas where the clearing sheet was laminated, and a coloured image of the test target was clearly visible.

The image was scanned in a Kodak RFS 35 mm film scanner and the resulting image file was digitally enhanced by increasing contrast, brightness, colour saturation and sharpness using Adobe Photoshop software, to give a brightly coloured and pleasing representation of the coloured test target.

What is claimed is:

1. A method of providing an image in an imagewise exposed photographic silver halide material comprising at least one silver halide emulsion layer, the method comprising developing the silver halide and fixing the remaining silver halide by contacting it with a molten composition comprising a silver halide complexing agent which is present in sufficient amount to render the silver halide substantially clear.

2. A method according to claim 1 wherein the silver halide and silver halide complexing agent are brought into contact at a temperature from 40 to 170° C.

3. A method according to claim 1 wherein the silver halide complexing agent is initially located in a separate fixer sheet

**36**

which is brought into contact with the photographic silver halide material.

4. A method according to claim 3 wherein the fixer sheet comprises a layer of the silver halide complexing agent in a polymeric binder on a support.

5. A method according to claim 1 wherein the silver halide complexing agent is initially located in an integral layer of the photographic silver halide material on the same side of the support as the silver halide photographic layer.

6. A method according to claim 1 wherein the silver complexing agent is a heterocyclic amine.

7. A method according to claim 6 wherein the heterocyclic amine is a substituted or unsubstituted imidazole, pyrazole or triazole.

8. A method according to claim 7 wherein the heterocyclic amine is imidazole or an alkyl substituted imidazole.

9. A method according to claim 1 further comprising the step of scanning the image formed to produce an electronic rendition of the image.

10. A method according to claim 9 further comprising digital processing of said rendition to manipulate, store, transmit, output, or display electronically said image.

\* \* \* \* \*